

## UNITED STATES PATENT OFFICE

2,149,257

METHOD FOR PRODUCTION OF BERYLLIUM  
COPPER ALLOYS

Herbert Gruber, Hanau-on-the-Main, Germany,  
assignor to Heraeus-Vacuumschmelze, A. G.,  
Hanau-on-the-Main, Germany

No Drawing. Application June 23, 1937, Serial  
No. 149,837. In Germany June 24, 1936

4 Claims. (Cl. 75—135)

I have heretofore proposed to produce beryllium alloys by dissolving carbon into an elementary constituent of the alloy to be formed, and the carbon containing metal bath is then brought to reaction in a vacuum or hydrogen atmosphere with beryllium oxide.

According to the present invention I may dispense with the previously molten copper bath entirely if desired.

Similarly, one need not operate with a rarefied chamber or a hydrogen atmosphere, but may proceed in air in a closed crucible.

I mix finely divided beryllium oxide or beryllium ore containing beryllium oxide, copper and carbon and bring the temperature up to about 2000° C. to 2300° C.

If desired, fluxes such as lime or calcium carbide may be used, although they are not necessary. The carbon may also be added in the form of its compounds, for instance, beryllium carbide. The copper may also be in the form of copper oxide. I may also produce other alloys of nickel, such as beryllium nickel or beryllium iron, in the same way, in which case I use an oxide of the metal to be alloyed with beryllium.

It is also possible for me to operate as low as about 1900° C. Here, however, I prefer, during the cooling period, to add known fluxes to the solidifying mixture, preferably halogen com-

pounds of alkali metals or earth alkali metals, these additions taking place at a temperature of between 1100° C. and 1800° C. and preferably between 1450° C. and 1550° C.

I claim:

1. The process of producing beryllium copper alloys which comprises supplying a mixture of finely divided beryllium oxide, copper and carbon, to a reaction temperature of from about 1900° C. to 2300° C.

2. The process of producing beryllium copper alloys which comprises supplying a mixture of finely divided beryllium oxide, copper and carbon, to a reaction temperature of from about 2000° C. to 2300° C.

3. The process of claim 1 characterized by the fact that fluxes are added to the reaction mixture during cooling when the mixture is at a temperature of from about 1100° C. to 1800° C. and preferably from 1450° C. to 1550° C.

4. The process of claim 1 characterized by the fact that a flux is added to the reaction mixture during cooling when the mixture is at a temperature of from about 1100° C. to 1800° C. and preferably from 1450° C. to 1550° C., said flux being chosen from the class consisting of halogen compounds of the alkali metals and of the alkali earth metals.

HERBERT GRUBER. 30